

Dec. 27, 1932.

B. STOCKFLETH

1,892,179

## METHOD OF MAKING BEARING SLEEVES

Filed Jan. 2, 1931



## UNITED STATES PATENT OFFICE

BERGER STOCKFLETH, OF NILES, MICHIGAN, ASSIGNOR, BY MESNE ASSIGNMENTS, TO THE CLEVELAND GRAPHITE BRONZE COMPANY, OF CLEVELAND, OHIO, A CORPORATION OF OHIO

## METHOD OF MAKING BEARING SLEEVES

Application filed January 2, 1931. Serial No. 506,196.

This invention relates to improvements in means and methods for making bi-metallic articles, such as lined bearing sleeves.

Such a sleeve consists of a relatively harder metal backing shell, such as steel, and a relatively softer bearing metal lining, such as Babbitt metal, and the invention relates particularly to improvements in the so-called pressure method of making or finishing such sleeves.

In the production of such a sleeve by the pressure method, a harder metal back is provided which is roughly of the desired dimensions and shape, though preferably thicker 15 radially and shorter both circumferentially and longitudinally than the finished back. Upon the inner surface of this rough back there is provided a layer of bearing metal preferably mechanically bonded to the back 20 by interlocking projections as well as by a suitable bonding coating, such as tin. This layer of bearing metal which is preferably Babbitt metal, is also roughly of the finished dimensions but is preferably also thicker 25 radially and shorter circumferentially and longitudinally than in the finished sleeve.

The sleeve blank thus provided, which is preferably less than a half cylinder, is placed in a die having a die opening of the shape and 30 dimensions of the outer surface of the finished sleeve, and a co-operating plunger is provided, the co-operating operative end of which has the shape and dimensions of the inner surface of the finished sleeve. The die 35 and plunger are so related that the ends of the die space are closed while at the longitudinal sides the space is open.

The plunger is forced into the die, thereby compressing the rough sleeve between the 40 plunger and the die, and pressure is applied sufficient to cause the lining and the back to be thinned radially and elongated circumferentially. Incidentally, the sleeve is also elongated longitudinally. The amount of metal 45 in the blank is preferably more than sufficient to form the finished sleeve, even when compressed, and the excess is forced out, that is, extruded through the openings or slots at the sides. The result of the application 50 of the heavy pressure applied is that the

rough bearing is shaped and sized accurately within the allowable tolerance and the sleeve is thereby completed except for the removal of the extruded portions along the longitudinal edges of the shell.

Preferably, the rough sleeve is heated to a temperature at which the bearing metal is malleable before being placed in the press, and also the dies may be maintained at a temperature preferably slightly less than the 55 melting point of the bonding metal. The pre-heating of the rough sleeves and the heating of the dies both assist in the perfection of the bond between the metals of the sleeves and in the reduction of the power used in the 60 pressing operation.

The invention will be best understood by reference to the accompanying drawing forming part of this specification and in which:—

Fig. 1 is a perspective view of a half-cylindrical bearing sleeve illustrating an article to which my invention applies and with parts broken away to best illustrate the invention;

Fig. 2 is an enlarged fragmentary section 75 on the line 2—2 of Fig. 1;

Fig. 3 is a diagrammatic sectional view of forming dies for forming the bearing sleeve, showing a sleeve in position to be pressed;

Fig. 4 is an enlarged view similar to Fig. 3, illustrating the finish of the pressing step; 80 and

Fig. 5 is an enlarged transverse section of the finished sleeve similar to the section shown in Fig. 4.

In said drawing, 1 illustrates a half cylindrical bearing comprising a backing shell 2 of harder metal, such as steel, brass or bronze, and an inner lining 3 of bearing metal, such 85 as Babbitt metal.

The lining 3 is bonded to the inner surface of the back. Preferably, in order to make this bond as perfect as possible, the inner surface of the back shell is roughened and bright 95 clean metal is presented over its whole inner surface, as indicated at 4. Then this surface, at least, of the back is tinned preferably by first dipping the back into a suitable acid bath to clean the back, then into a pot of 100

melted tin. The tin coating on the inside which is very thin is indicated at 5.

After the back is thus prepared, the Babbitt metal lining is added by some method which causes it to be bonded to the back through the tin bond and the roughening of the back. This may be accomplished by the method disclosed in Patent No. 1,803,513 issued to me May 5, 1931, or by some other suitable method.

Both the backing shell 2 and the lining 3 are slightly thicker radially and shorter circumferentially than the dimensions desired in the completed bearing sleeve. This is for the finishing step in completing the sleeve.

The finishing step is illustrated in Figs. 3 and 4, wherein 6 is a die block having a die opening 7 of the shape and dimensions of the outer or convex surface of the finished bearing, and 9 is a plunger having a lower end 10 for co-operation with the die member 6 to form the inner or concave surface 11 of the finished sleeve. The end 10 of the plunger 9 is accurately of the size and form desired for the inner concave surface 11 of the finished sleeve.

As shown in Fig. 3, the rough sleeve is preferably not quite a half circle, as indicated by the clearance spaces 12 at its edges.

Preferably, as stated, the rough sleeves are pre-heated to a temperature approximately the melting point of the bonding metal before they are placed in the press and the dies are preferably maintained at approximately the same temperature by any suitable means, such as electrically heated elements 13 arranged in suitable openings 14 in the die members 6 and 9.

The pressure method of sizing and finishing the bearing sleeve consists in subjecting the rough sleeves to an enormous pressure radially in suitable dies, such as those shown at 6 and 9, sufficient to actually compress and thin the sleeve radially and cause it to be squeezed out and elongated circumferentially. Such manipulation of the sleeve in the forming pressure results in many advantageous features.

Both the lining and the backing are compressed beyond their respective elastic limits and are consequently more solid or dense than before the operation. This is of benefit in causing the bearing sleeve to transmit heat more effectively outwardly in use, resulting in a cooler running bearing. This compression of the metal of the sleeve goes far beyond any compressive forces to which it may be subjected to in use, and consequently the sleeve is more permanent in form. Furthermore, by such pressure method the sleeves are accurately sized within the allowable tolerance and they ordinarily do not need any sizing by any cutting or machining methods.

The bearing metal, such as Babbitt metal,

being much softer and more easily thinned out than the metal of the back, some retarding means is necessary to prevent the squeezing out of the bearing metal in considerable advance of the thinning out of the back. Such relative flow is especially detrimental as the flowing of the lining metal on the back tends to disrupt and destroy the bond between the back and the lining.

70

Many methods have been devised for improving the bond between the lining and the back but, so far as I am aware, none of these methods have satisfactorily withstood the strain incident to the pressure method of forming and finishing. By means of this present method, however, I am enabled to attain a substantially perfect bond between the back and the lining in bearing sleeves finished by the pressure method.

75

In applying forming pressure to the sleeve by the die and punch method illustrated, it is obvious that when pressure is applied sufficient to cause the lining metal to be squeezed out of the die space through the longitudinal slots 12 between the sides of the die and plunger, that there will be more or less drag on the backing shell and if this drag can be made great enough, the two parts will be substantially equally elongated circumferentially. I increase this drag by two means; first, by the very thorough roughening and cleaning of the inside of the backing shell preferably by what is known as the "shot blasting" or deep etching; and second, by making the lining of Babbitt metal relatively thin, and applying it in such a manner that it is not only mechanically bonded to the back through its roughened surface, but also molecularly bonded through the medium of the bonding metal as explained, preferably tin.

80

Such thorough and complete bonding of the lining to the back, especially when the lining is relatively thin, results in the substantially equal elongation of the back and the lining, and no mechanical means is necessary to prevent the advance or excess extrusion of the lining metal.

90

A relative proportion as to thickness between the back and lining which has proven successful in this method is substantially 1 to 3 or more, that is, the lining is substantially one third or less as thick as the back.

95

As illustrated in Fig. 4, the lining metal may be extruded to a slight degree faster than the back, as illustrated by the outwardly curved extruded portions 15, but this is not sufficient to disrupt the bond between the lining and the back.

100

To complete the bearing sleeve, these extruded parts 15 are removed by any suitable method, as indicated by the dotted lines in Fig. 5.

105

Unless some hindering means are provided, the softer bearing metal will be thinned out and extruded in advance of the backing metal.

110

115

120

125

130

There are two causes tending to prevent the advance thinning and extrusion of the Babbitt metal; these are the drag of the bearing metal on the plunger and the drag of the bearing metal on the back. The bearing metal which lies between the outer and inner surfaces of the lining will be held against extrusion by the molecular forces in the lining metal as augmented by the drag on the inner and outer surfaces of the lining, consequently, I make the lining relatively thin and thus prevent the advance extrusion of the lining metal to any substantial extent.

In other words, I so proportion the thickness of the lining and back that the two metals are substantially equally extruded from the dies. It is to be understood, of course, that a thorough mechanical bonding of the lining to the back as well as a bonding by means of a suitable bonding metal is an advantage in obtaining the results desired.

It has been found in practice that if the lining is not more than approximately  $3/64''$  thick it will not be extruded in advance of the backing metal.

The invention resides in a bearing sleeve blank having a harder metal back and a bearing metal lining bonded to the back and so proportioned in thickness to the thickness of the back that when the blank is subjected to radial pressure in suitable forming dies for the purpose of sizing and finishing the sleeve, the lining is not thinned to any substantial extent in advance of the back but for all practicable purposes the back and lining are simultaneously thinned.

The invention also resides in the herein described pressure method of forming and sizing bi-metal bearing sleeves and which includes the provision of blanks for formation by the pressure method, the blank comprising harder metal backs and bearing metal linings bonded thereto and so proportioned as to thickness that the drag of the lining on the forming plunger and on the back shell to which it is bonded is sufficient to prevent any substantial thinning of the lining in advance of the back.

As many modifications of the invention will readily suggest themselves to one skilled in the art, I do not limit or confine the invention to the specified sequence or steps or specific construction herein described except within the scope of the appended claims.

55 I claim:

1. The herein described method of making a bi-metal bearing sleeve of the kind described, which consists in first making a bi-metal blank for the sleeve, the blank consisting of a harder, tougher metal back and a relatively softer bearing metal lining, the lining both mechanically and molecularly bonded to the back and the lining being relatively thin and subjecting the blank to sufficient pressure applied substantially radial-

ly thereto in suitable dies, to thin the sleeve radially and cause substantially equal elongation of the metals of the sleeve in a direction substantially parallel to the die surfaces.

2. The invention as defined in claim 1 the elongation of the metals being most pronounced in a circumferential direction.

3. The invention as defined in claim 1, the space between the dies provided with an outlet permitting extrusion of the surplus material, the outlet being so placed and large enough so that both the lining and the back will be extruded therethrough, and the lining and back so proportioned as to thickness that they are substantially equally extruded.

4. The herein described method of making bearing sleeves which includes the provision of a substantially half-cylindrical roughly sized blank, consisting of a relatively harder, tougher metal back and a relatively softer and more ductile bearing metal lining, and pressing the blank between suitable die members, the applied pressure being sufficient to thin the sleeve radially and elongate it in a direction substantially parallel with the die surface, and the bearing metal lining being thin enough so that the two metals are substantially equally elongated.

5. The herein described method of making a bi-metal bearing sleeve of the kind described, which consists in first making a bi-metal blank for the sleeve roughly formed to shape and consisting of a back of harder tougher metal such as steel, and a bearing metal lining secured to the back by a suitable bonding metal, heating the blank to approximately the melting point of the bonding metal, and subjecting the sleeve, in such heated condition, to pressure applied substantially radially thereto, the applied pressure being sufficient to cause the sleeves to be thinned radially and the substantially equal elongation of the metals of the sleeve substantially parallel with the die surfaces.

6. The invention as defined in claim 5 and maintaining the dies heated to approximately the melting temperature of the bonding metal.

In testimony whereof, I have hereunto set my hand this fifteenth day of December, 1930,

BERGER STOCKFLETH.

120

125

130